

Feb. 11, 1936.

D. D. UONG

2,030,483

## METHOD FOR THE MANUFACTURE OF COATED PAPER

Filed April 1, 1933

2 Sheets-Sheet 1



Inventor  
Dong D. Wong  
By Attorney

Saintgate Fay. Hawley

Feb. 11, 1936.

D. D. UONG

2,030,483

METHOD FOR THE MANUFACTURE OF COATED PAPER

Filed April 1, 1933

2 Sheets-Sheet 2



## UNITED STATES PATENT OFFICE

2,030,483

METHOD FOR THE MANUFACTURE OF  
COATED PAPERDiong D. Uong, Fitchburg, Mass., assignor to  
Fitchburg Paper Company, Fitchburg, Mass., a  
corporation of Massachusetts

Application April 1, 1933, Serial No. 663,966

1 Claim. (Cl. 92—40)

This invention relates to the manufacture of paper presenting a coated surface at one or both sides thereof. Such coated papers are commonly produced by the application of a suitable coating material to previously formed paper, and in the usual commercial practice a liquid coating material has been applied to the paper after the paper has been dried and removed from the paper making machine. Such application of liquid coating material to substantially dry paper involves a separate and additional coating operation as well as a second drying operation, all at substantial additional expense.

It is the general object of my invention to produce a coated paper by the application of a coating material in powdered form to a web of paper while it is still in the paper making machine and before the drying thereof is completed.

Preferably I apply the powder to the web at a point where the web still contains a substantial amount of water, a condition found at the suction boxes and to a less extent at the press rolls. It may at times, however, be desirable to apply the powdered coating material even later in the paper making process, as for instance at a point between sections of drying cylinders.

In any event, the powdered coating material is to be applied uniformly to the paper web while it still contains sufficient moisture to coat with the powdered material and produce an effective coating on the paper.

A further object of my invention is to provide improved mechanism for thus uniformly applying a powdered coating material to a paper web in a paper making machine.

My invention further relates to arrangements and combinations of parts which will be herein-after described and more particularly pointed out in the appended claim.

A preferred form of the invention is shown in the drawings, in which

Fig. 1 is a diagrammatic side elevation of portions of a paper making machine having my invention applied thereto;

Fig. 2 is a sectional side elevation of a preferred form of mechanism for applying the powdered coating material to the moist web;

Fig. 3 is a sectional elevation of the coating-applying mechanism, taken along the line 3—3 in Fig. 2;

Fig. 4 is a detail side elevation of a portion of one of the feeding plates;

Fig. 5 is an end view, looking in the direction of the arrow 5 in Fig. 4, and

Fig. 6 is a detail view, looking in the direction of the arrow 6 in Fig. 5.

Referring to Fig. 1, I have shown portions of a paper making machine of a usual type and having a Fourdrinier section A, a press roll section B and a drying section C. The Fourdrinier section A comprises a fine mesh wire screen apron or conveyor 10 on which the paper material or pulp is deposited and through which a portion of the water escapes or is sucked away.

The apron 10 and partially formed paper web W passes over a series of suction boxes 11, under a dandy roll 12, and around a larger or couch roll 13. The partially formed paper web W then passes between successive pairs of press rolls 14, 15 and 16 in the press roll section B, after which the web passes around a series of drying rolls or cylinders 20 in the drying section C, the cylinders 20 being of relatively large size and steam-heated to remove a substantial portion of the moisture still remaining in the web W.

The paper-making machine thus briefly described is of a usual commercial type and in itself constitutes no part of my present invention, which relates particularly to the mechanism M for applying coating material in powdered form to the paper web W as it passes through the paper-making machine.

The location of the mechanism M in the paper-making machine is subject to somewhat wide variation but as at present practiced, I preferably mount the mechanism M so that the powdered material is applied to the paper web W as it passes over the first pair of suction boxes 11, at which point the paper web may comprise eighty percent or more of water.

While the position above the suction boxes is at present favored, the mechanism M may, if desired, be so mounted as to deliver the powdered coating material to the paper web W as it passes through the press roll section B of the machine. Such a location is indicated in dotted lines in Fig. 1, the coating mechanism M' being positioned to apply the coating material to the web W as it passes from the first pair of press rolls 14 to the second pair of press rolls 15, at which point the web W contains substantially less moisture than at the suction boxes.

I may also position the coating mechanism entirely beyond the press roll section, as indicated in dotted lines at M<sup>2</sup> in Fig. 1. Under certain conditions it is desirable to locate the coating mechanism between sections of drying cylinders, as indicated in dotted lines at M<sup>3</sup> in Fig. 1, at

which point the moisture content of the paper web may be as low as twenty percent.

The location of the coating mechanism will be selected with reference to the paper stock, the 5 coating material, the type of surface to be produced, and other operating conditions.

In Figs. 2 to 6 I have shown a form of coating mechanism M which is well adapted for applying powdered coating material to the paper web W.

10 As shown in the drawings, the coating mechanism M comprises a casing 22 mounted on suitable supporting frame members 23 adapted to be easily secured to the main frame of the paper-making machine at a desired location.

15 A pair of distributing rolls 24 and 25 are supported in bearings 26 on the frame members 23 and are rotated by the driving belt 27 in the direction of the arrows a in Fig. 2. A hopper 30 is mounted above the casing 22 and is provided 20 with feed plates 32, adjustably secured to blocks 34 and 35 which in turn are mounted on pairs of slide bars 36.

The blocks 34 at each side of the hopper are 25 connected by links 40 and 41 to eccentric pins 42 rotated with a pulley 43 by a belt 44. As the pulley 43 is rotated, it will be obvious that the feed plates 32 are given slight reciprocating movements in reversed directions, thus tending to evenly distribute the powdered material 30 lengthwise of the plates and to feed the material downward through the relatively narrow opening between the lower edges of the feed plates 32. The width of this opening may be adjusted by 35 adjusting the plates 32 in the blocks 34 and 35, for which purpose adjusting screws 45 are provided.

The feed plates 32 converge downward as 40 shown in Fig. 2, and the lower edges of the plates are preferably beveled as indicated at 46 in Fig. 5. The lower portions of the plates 32 are also 45 preferably grooved as indicated at 47 in Figs. 4 and 6, and the beveled edges 46 are preferably provided with finer grooves as indicated at 48 in Figs. 4 and 6. As the plates 32 are relatively reciprocated, the grooved lower portions of the plates tend to pulverize the powdered coating material, should any lumps or hard portions occur therein.

By the use of these reciprocating grooved feed plates a fine uniform stream of powdered material is delivered to the roll 24 within the casing 22, and a considerable portion of this material is passed along by the roll 24 to the roll 25, as indicated at Fig. 2.

After leaving the roll 25, the powdered material circulates in different directions within the casing 22 and is finally deposited in a substantially uniform manner on the moist surface of the paper web W. The rolls 24 and 25 are preferably provided with knurled surfaces as indicated in Fig. 3 for more effectively advancing and distributing the powdered material.

It will be evident from the foregoing description that the mechanism M for applying the powdered material to the paper web is a self-contained unit which may be readily mounted in any convenient position in a paper-making machine, as indicated at M, M', M<sup>2</sup> and M<sup>3</sup> in Fig. 1, the particular position selected depending 15 on the nature of the product and desired coating and on the operating conditions.

It is deemed essential that the paper web should have sufficient substance so that the powdered material will remain largely on the surface of 20 the web, and furthermore that the web shall contain sufficient moisture to coat with the powdered material in producing an effective coating. Under ordinary conditions the moisture content will run from twenty to ninety percent 25 in the web at the point of powder application.

The powdered material itself may be varied to suit operating conditions and the particular type of coating desired, but will commonly consist largely of an adhesive material mixed with some 30 form of pigment of different colors.

Having thus described my invention and the advantages thereof, I do not wish to be limited to the details herein disclosed, otherwise than as set forth in the claim, but what I claim is:— 35

The method of coating paper which comprises removing a portion only of the moisture from a paper web in a paper machine having forming wires and a pressing section, applying a coating of moisture-reactive coating material in dry powdered form to the paper web after said web has left the forming wires and at a point adjacent the pressing section, allowing said powdered coating material to coat with the still substantially moist paper web, and thereafter drying and removing additional moisture from said web and causing said previously powdered material to form a relatively smooth surface on the paper prior to leaving said machine, all of said operations being performed successively as parts of 40 a continuous paper-making process. 45

DIONG D. UONG.